



US010813381B2

(12) **United States Patent**  
**Klipfel et al.**

(10) **Patent No.:** **US 10,813,381 B2**  
(45) **Date of Patent:** **Oct. 27, 2020**

(54) **HOMOGENIZED TOBACCO MATERIAL AND METHOD OF PRODUCTION OF HOMOGENIZED TOBACCO MATERIAL**

(71) Applicant: **PHILIP MORRIS PRODUCTS S.A.**, Neuchatel (CH)

(72) Inventors: **Yorick Klipfel**, St. Saphorin-sur-Morge (CH); **Johannes Petrus Maria Pijnenburg**, Neuchatel (CH); **Michael Elliott Doyle**, Ridgeway, VA (US); **Juan David Manzur Bedoya**, Lutry (CH); **Pascal Rausis**, Colombier (CH); **Marine Jarriault**, Bern (CH)

(73) Assignee: **Philip Morris Products S.A.**, Neuchatel (CH)

(\*) Notice: Subject to any disclaimer, the term of this patent is extended or adjusted under 35 U.S.C. 154(b) by 120 days.

(21) Appl. No.: **15/503,808**

(22) PCT Filed: **Sep. 9, 2015**

(86) PCT No.: **PCT/EP2015/070655**

§ 371 (c)(1),

(2) Date: **Feb. 14, 2017**

(87) PCT Pub. No.: **WO2016/050471**

PCT Pub. Date: **Apr. 7, 2016**

(65) **Prior Publication Data**

US 2017/0273347 A1 Sep. 28, 2017

(30) **Foreign Application Priority Data**

Sep. 30, 2014 (EP) ..... 14187203

(51) **Int. Cl.**

**A24B 3/14** (2006.01)

**A24B 15/14** (2006.01)

**A24B 15/167** (2020.01)

(52) **U.S. Cl.**

CPC ..... **A24B 3/14** (2013.01); **A24B 15/14** (2013.01); **A24B 15/167** (2016.11)

(58) **Field of Classification Search**

None

See application file for complete search history.

(56) **References Cited**

**U.S. PATENT DOCUMENTS**

4,306,578 A 12/1981 Schmidt  
4,972,854 A \* 11/1990 Kiernan ..... **A24B 3/14**  
131/353

(Continued)

**FOREIGN PATENT DOCUMENTS**

CN 203281455 11/2013  
CN 103445285 12/2013

(Continued)

**OTHER PUBLICATIONS**

Office Action issued in China for Application No. 20150049816.6 dated Aug. 7, 2018 (21 pages). English translation included.

(Continued)

*Primary Examiner* — Michael H. Wilson

*Assistant Examiner* — Katherine A Will

(74) *Attorney, Agent, or Firm* — Muetting Raasch Group

(57) **ABSTRACT**

The invention relates to a method for the preparation of a homogenized tobacco material, said method comprising: —pulping and refining cellulose fibres to obtain fibres having a mean size comprised between about 0.2 millimetres and about 4 millimetres; —grinding a blend of tobacco of one or more tobacco types to a tobacco powder having a mean size comprised between about 0.03 millimetres and about 0.12 millimetres; —combining the pulp with the tobacco powder blend of different tobacco types and with a binder in an amount comprised between about 1 percent and about 5 percent in dry weight basis of the total weight

(Continued)



of the homogenized tobacco material, so as to form a slurry;—homogenizing the slurry; and—forming the homogenized tobacco material from the slurry.

**17 Claims, 7 Drawing Sheets**

(56)

**References Cited**

**U.S. PATENT DOCUMENTS**

9,439,451 B2 9/2016 Volgger  
2012/0006343 A1\* 1/2012 Renaud ..... A24B 15/12  
131/280

**FOREIGN PATENT DOCUMENTS**

|    |           |         |
|----|-----------|---------|
| CN | 203340993 | 12/2013 |
| CN | 104053369 | 9/2014  |
| CN | 103462203 | 7/2015  |
| CN | 103393210 | 9/2015  |
| CN | 103416839 | 6/2016  |
| EP | 2617299   | 7/2013  |
| EP | 2526787   | 12/2017 |
| GB | 815315    | 6/1959  |
| GB | 961866    | 6/1964  |
| GB | 0565360   | 10/1993 |

**OTHER PUBLICATIONS**

PCT Search Report and Written Opinion for PCT/EP2015/070655  
dated Nov. 3, 2015 (11 pages).  
Office Action issued in China for Application No. 20150049816.6  
dated Dec. 4, 2017 (22 pages). English translation included.

\* cited by examiner





FIG. 2



FIG. 3



FIG. 4



FIG. 5





## HOMOGENIZED TOBACCO MATERIAL AND METHOD OF PRODUCTION OF HOMOGENIZED TOBACCO MATERIAL

This application is a U.S. National Stage Application of International Application No. PCT/EP2015/070655, filed Sep. 9, 2015, which was published in English on Apr. 7, 2016 as International Publication No. WO 2016/050471 A1. International Application No. PCT/EP2015/070655 claims priority to European Application No. 14187203.6 filed Sep. 30, 2014.

This invention relates to a process for producing homogenized tobacco material. In particular, the invention relates to a process for producing homogenized tobacco material for use in an aerosol-generating article such as, for example, a cigarette or a “heat-not-burn” type tobacco containing product.

Today, in the manufacture of tobacco products, besides tobacco leaves, also homogenized tobacco material is used. This homogenized tobacco material is typically manufactured from parts of the tobacco plant that are less suited for the production of cut filler, like, for example, tobacco stems or tobacco dust. Typically, tobacco dust is created as a side product during the handling of the tobacco leaves during manufacture.

The most commonly used forms of homogenized tobacco material are reconstituted tobacco sheet and cast leaf. The process to form homogenized tobacco material sheets commonly comprises a step in which tobacco dust and a binder are mixed to form a slurry. The slurry is then used to create a tobacco web, for example by casting a viscous slurry onto a moving metal belt to produce so called cast leaf. Alternatively, a slurry with low viscosity and high water content can be used to create reconstituted tobacco in a process that resembles paper-making. Once prepared, homogenized tobacco webs may be cut in a similar fashion as whole leaf tobacco to produce tobacco cut filler suitable for cigarettes and other smoking articles. The function of the homogenized tobacco for use in conventional cigarettes is substantially limited to physical properties of tobacco, such as filling power, resistance to draw, tobacco rod firmness and burn characteristics. This homogenized tobacco is typically not designed to have taste impact. A process for making such homogenized tobacco is for example disclosed in European Patent EP 0565360.

Homogenized tobacco material that is intended for use as an aerosol-forming substrate of a heated aerosol-generating article of the “heat-not-burn” type tends to have a different composition to homogenized tobacco intended for use as filler in conventional cigarettes. In a heated aerosol-generating article, an aerosol-forming substrate is heated to a relatively low temperature, in order to form an aerosol. Further, the tobacco present in the homogenized tobacco material is typically the only tobacco, or includes the majority of the tobacco, present in the aerosol-generating article.

During the production of aerosol generating articles comprising homogenized tobacco material from a homogenized tobacco material web, the homogenized tobacco web is typically required to withstand some physical handling like for example, wetting, conveying, drying and cutting. It would be therefore desirable to provide a homogenized tobacco web that is adapted to withstand such handling with no or minimal impact on the quality of the final tobacco material. In particular, it would be desirable, that the homogenized tobacco material web shows little complete or partial ripping. A ripped homogenized tobacco web could lead to the loss of tobacco material during manufacture. Also, a

partially or completely ripped homogenized tobacco web may lead to machine downtime and waste during machine stops and ramp up.

Therefore, there is a need for a new method of preparing a homogenized tobacco web for the use in heated aerosol-generating articles of the “heat-not-burn” type that is adapted to the different heating characteristics and aerosol forming needs of such a heated aerosol-generating article. Such a homogenized tobacco web should further be adapted to withstand the required manufacturing processes.

According to a first aspect, the invention relates to a method for the production of a homogenized tobacco material. The method includes the steps of pulping and refining cellulose fibres so as to form a pulp and grinding a blend of tobacco of one or more tobacco types. In a further step, a slurry is formed by combining the tobacco blend powder of different tobacco types with the pulp and a binder. A further step comprises homogenizing the slurry, and forming a homogenized tobacco material from the slurry. According to 15 the invention, the pulping and refining step outputs cellulose fibres having a mean size between about 0.2 millimetres and about 4 millimetres. The grinding step produces a tobacco powder blend having a mean size comprised between about 0.03 millimetres and about 0.12 millimetres. The binder is 20 added in the slurry in an amount between about 1 percent and about 5 percent in dry weight basis of the total weight of the homogenized tobacco sheet.

The term “homogenized tobacco material” is used throughout the specification to encompass any tobacco material formed by the agglomeration of particles of tobacco material. Sheets or webs of homogenized tobacco are formed in the present invention by agglomerating particulate tobacco obtained by grinding or otherwise powdering of one or both of tobacco leaf lamina and tobacco leaf stems.

In addition, homogenized tobacco material may comprise a minor quantity of one or more of tobacco dust, tobacco fines, and other particulate tobacco by-products formed during the treating, handling and shipping of tobacco.

As the tobacco present in the homogenized tobacco material constitutes substantially the only—or the majority of—tobacco present in the aerosol-generating article, the impact on the characteristics of the aerosol, such as its flavour, derives predominantly from the homogenized tobacco material. It is preferred that the release of substances 40 from the tobacco present in the homogenized tobacco material is simplified, in order to optimize use of tobacco. According to the invention, the tobacco powder is—at least for a fraction of the total tobacco powder amount—of the same size or below the size of the tobacco cell structure. It 45 is believed that fine grinding tobacco to about 0.05 millimetres can advantageously open the tobacco cell structure and in this way the aerosolization of tobacco substances from the tobacco itself is improved. Examples of substances for which the aerosolization may be improved by providing 50 tobacco powder with a mean powder size between about 0.03 millimetres and about 0.12 millimetres are pectin, nicotine, essential oils and other flavours. In the following, the term “tobacco powder” is used through the specification to indicate tobacco having a mean size between about 0.03 millimetres and about 0.12 millimetres.

The same mean size of the tobacco powder between about 0.03 millimetres and about 0.12 millimetres may also improve the homogeneity of the slurry. Too big tobacco particles, that is, tobacco particles bigger than about 0.15 millimetres, may be the cause of defects and weak areas in the homogenized tobacco web which is formed from the slurry. Defects in the homogenized tobacco web may reduce

the tensile strength of the homogenized tobacco web. A reduced tensile strength may lead to difficulties in subsequent handling of the homogenized tobacco web in the production of the aerosol-generating article and could for example cause machine stops. Additionally, an inhomogeneous tobacco web may create unintended difference in the aerosol delivery between aerosol generating articles that are produced from the same homogenized tobacco web. Therefore, a tobacco having relatively small mean particle size is desired as a starting tobacco material to form the slurry to obtain acceptable homogenized tobacco material for aerosol-generating articles. Too small tobacco particles increases the energy consumption required in the process for their size reduction without adding advantages for this further reduction.

A reduced tobacco powder mean size is also beneficial due to its effect on reducing the viscosity of the tobacco slurry, thereby allowing a better homogeneity. However, at the size between about 0.03 millimetres and about 0.12 millimetres, the tobacco cellulose fibres within the tobacco powder are substantially destroyed. Therefore, the tobacco cellulose fibres within the tobacco powder may have only a very small contribution to the tensile strength of the resulting homogenized tobacco web. Conventionally, this is compensated by the addition of binders. Nevertheless, there is a practical limit to the amount of binders that may be present in the slurry and hence in the homogenized tobacco material. This is due to the tendency of the binders to gel when coming in contact with water. Gelling strongly influences the viscosity of the slurry, which in turn is an important parameter of the slurry for subsequent web manufacturing processes, like for example casting. It is therefore preferred to have a relatively low amount of binder in the homogenized tobacco material. According to the invention, the quantity of binder added to the blend of one or more tobacco types is comprised between about 1 percent and about 5 percent in dry weight of the slurry. The binder used in the slurry can be any of the gums or pectins described herein. The binder may ensure that the tobacco powder remains substantially dispersed throughout the homogenized tobacco web. For a descriptive review of gums, see Gums And Stabilizers For The Food Industry, IRL Press (G. O. Phillip et al. eds. 1988); Whistler, Industrial Gums: Polysaccharides And Their Derivatives, Academic Press (2d ed. 1973); and Lawrence, Natural Gums For Edible Purposes, Noyes Data Corp. (1976).

Although any binder may be employed, preferred binders are natural pectins, such as fruit, citrus or tobacco pectins; guar gums, such as hydroxyethyl guar and hydroxypropyl guar; locust bean gums, such as hydroxyethyl and hydroxypropyl locust bean gum; alginate; starches, such as modified or derivitized starches; celluloses, such as methyl, ethyl, ethylhydroxymethyl and carboxymethyl cellulose; tamarind gum; dextran; pullulan; konjac flour; xanthan gum and the like. The particularly preferred binder for use in the present invention is guar.

Although on one hand the relatively small tobacco powder mean size and the reduced amount of binder may result in a very homogeneous slurry and then in a very homogeneous homogenized tobacco material, on the other hand the tensile strength of the homogenized tobacco web obtained from this slurry may be relatively low and potentially insufficient to adequately withstand the forces acting on the homogenized tobacco material during processing.

According to the invention, cellulose fibres are introduced in the slurry. Those cellulose fibres are added to the cellulose fibres present within the tobacco itself, that is to say, the

cellulose fibres herein mentioned are fibres other than the fibres naturally present in the tobacco blend powder and they are called in the following "added cellulose fibres". The introduction of cellulose fibres in the slurry increases the tensile strength of the tobacco material web, acting as a strengthening agent. Therefore, adding cellulose fibres in addition to those already present in the tobacco may increase the resilience of the homogenized tobacco material web. This supports a smooth manufacturing process and subsequent handling of the homogenized tobacco material during the manufacture of aerosol generating articles. In turn, this can lead to an increase in production efficiency, cost efficiency, reproducibility and production speed of the manufacture of the aerosol-generating articles and other smoking articles.

Cellulose fibres for including in a slurry for homogenized tobacco material are known in the art and include, but are not limited to: soft-wood fibres, hard wood fibres, jute fibres, flax fibres, tobacco fibres and combination thereof. In addition to pulping, the cellulose fibres might be subjected to suitable processes such as refining, mechanical pulping, chemical pulping, bleaching, sulphate pulping and combination thereof.

Fibres particles may include tobacco stem materials, stalks or other tobacco plant material. Preferably, cellulose-based fibres such as wood fibres comprise a low lignin content. Alternatively fibres, such as vegetable fibres, may be used either with the above fibres or in the alternative, including hemp and bamboo.

One relevant factor in the added cellulose fibres is the cellulose fibre length. Where the cellulose fibres are too short, the fibres would not contribute efficiently to the tensile strength of the resulting homogenized tobacco material. Where the cellulose fibres are too long, the cellulose fibres would impact the homogeneity in the slurry and in turn may create inhomogeneities and other defects in the homogenized tobacco material, in particular for thin homogenized tobacco material, for example with a homogenized tobacco material with a thickness of several hundreds of micrometres.

According to the invention, the size of added cellulose fibres in a slurry comprising tobacco powder having a mean size between about 0.03 millimetres and about 0.12 millimetres and a quantity of binder between about 1 percent and about 5 percent in dry weight of the slurry, is advantageously between about 0.2 millimetres and about 4 millimetres.

Preferably, the mean size of the cellulose fibres is between about 1 millimetre and about 3 millimetres. Preferably, this further reduction is obtained by means of a refining step. In the present specification, the fibre "size" means the fibre length, that is, the fibre length is the dominant dimension of the fibre. Thus, mean fibre size has the meaning of mean fibre size length. The mean fibre length is the mean fiber length per a given number of fibers, excluding fibers having a length below about 200 microns or above about 10,000 microns and excluding fibres having a width below about 5 microns or above about 75 microns. Further, preferably, according to the invention, the amount of the cellulose fibres added to the cellulose fibres present in the tobacco powder blend is comprised between about 1 percent and about 3 percent in dry weight basis of the total weight of the slurry.

These values of the ingredients of the slurry have shown to improved tensile strength while maintaining a high level of homogeneity of the homogenized tobacco material compared to homogenized tobacco material that only relies on binder to address tensile strength of the homogeneous tobacco web. At the same time, cellulose fibres having a mean size, for example a mean length, between about 0.2

millimetres and about 4 millimetres do not significantly inhibit the release of substances from the fine ground tobacco powder when the homogenized tobacco material is used as an aerosol generating substrate of an aerosol generating article. According to the invention, a relatively fast and reliable manufacturing process of homogenized tobacco web can be obtained, as well as a substrate that is adapted to release a highly reproducible aerosol.

Preferably, the step of pulping and refining comprises a step of fibrillating the cellulose fibres at least in part. The cellulose fibres herein considered which are fibrillated are those added to the cellulose fibres contained in the tobacco blend. The fibrillation of the added fibres may improve the strengthening of the homogenized tobacco webs. To obtain fibres' fibrillation, the fibres are for example subjected to mechanical friction, shearing and compression forces. Fibrillation may include the partial delamination of the cell walls of the cellulose fibres, resulting in a microscopically hairy appearance of the wetted cellulose fibres' surfaces. The "hairs" are also called microfibrils. The smallest microfibrils may be as small as individual cellulose chains. Fibrillation tends to increase the relative bonded area between cellulose fibres after the slurry has been dried, increasing the tensile strength of the homogenized tobacco web.

Preferably, the method comprises the step of vibrating the slurry. Vibrating the slurry, that is for example vibrating a tank or silo where the slurry is present, may help the homogenization of the slurry. Less mixing time may be required to homogenize the slurry to the target value optimal for casting if together with mixing also vibrating is performed.

Advantageously, the step of pulping and refining comprises the steps of forming a concentrated pulp wherein the amount of the cellulose fibres is between about 3 percent and about 5 percent of the total weight of the concentrated pulp; and diluting said concentrated pulp wherein the amount of cellulose fibres is below about 1 percent of the total weight of the diluted pulp. The cellulose fibres present in the pulp are added to the cellulose fibres naturally present in the tobacco blend to form the slurry. For example, the concentrated pulp may be diluted by a factor of between about 4 and about 20 with water.

The pulp is formed by adding together the cellulose fibres and water. The water is preferably added in two separate steps. First the pulp is produced mixing together the cellulose fibres and a first amount of water so that the amount of cellulose fibres in the total weight of the pulp is comprised between about 3 percent and about 5 percent. This concentrated pulp is then preferably stored and diluted until it is added to the other ingredients forming the slurry. In this way the amount of water that is introduced in the slurry can be easily controlled.

Advantageously, the method comprises the step of adding an aerosol-former to the slurry. Suitable aerosol-formers for inclusion in slurry for webs of homogenised tobacco material are known in the art and include, but are not limited to: monohydric alcohols like menthol, polyhydric alcohols, such as triethylene glycol, 1,3-butanediol and glycerine; esters of polyhydric alcohols, such as glycerol mono-, di- or triacetate; and aliphatic esters of mono-, di- or polycarboxylic acids, such as dimethyl dodecanedioate and dimethyl tetradecanedioate. For example, where the homogenized tobacco material according to the specification is intended for use as aerosol-forming substrates in heated aerosol-generating articles, webs of homogenised tobacco material may have an aerosol-former content of between about 5

percent and about 30 percent by weight on a dry weight basis. Homogenized tobacco webs intended for use in electrically-operated aerosol-generating system having a heating element may preferably include an aerosol former of between about 5 percent to about 30 percent on dry weight basis of the homogenized tobacco material, preferably between about 10 percent to about 25 percent on dry weight basis of the homogenized tobacco material. For homogenized tobacco webs intended for use in electrically-operated aerosol-generating system having a heating element, the aerosol former may preferably be glycerol.

In a preferred embodiment, the step of forming a homogenized tobacco material from the slurry comprises the steps of casting a web of the slurry, and drying the cast web.

15 A web of homogenized tobacco material is preferably formed by a casting process of the type generally comprising casting a slurry prepared as above described on a support surface. Preferably, the cast web is then dried to form a web of homogenized tobacco material and it is then removed 20 from the support surface.

25 Preferably, the moisture of said cast tobacco material web at casting is between about 60 percent and about 80 percent of the total weight of the tobacco material at casting. Preferably, the method for production of a homogenized tobacco material comprises the step of drying said cast web, winding said cast web, wherein the moisture of said cast web at winding is between about 7 percent and about 15 percent of the total weight of the tobacco material web. Preferably, the moisture of said homogenized tobacco web at winding is 30 between about 8 percent and about 12 percent of the total weight of the homogenized tobacco web.

35 Preferably, said step of blending tobacco of one or more tobacco type comprises blending one or more of the following tobaccos: bright tobacco, dark tobacco; aromatic tobacco; filler tobacco. In the present invention, the homogenized tobacco material is formed by tobacco lamina and stem of different tobacco types, which are properly blended. With the term "tobacco type" one of the different varieties of 40 tobacco is meant. With respect to the present invention, these different tobacco types are distinguished in three main groups of bright tobacco, dark tobacco and aromatic tobacco. The distinction between these three groups is based on the curing process the tobacco undergoes before it is further processed in a tobacco product.

45 Bright tobaccos are tobaccos with a generally large, light coloured leaves. Throughout the specification, the term "bright tobacco" is used for tobaccos that have been flue cured. Examples for bright tobaccos are Chinese Flue-Cured, Flue-Cured Brazil, US Flue-Cured such as Virginia tobacco, Indian Flue-Cured, Flue-Cured from Tanzania or other African Flue Cured. Bright tobacco is characterized by a high sugar to nitrogen ratio. From a sensorial perspective, bright tobacco is a tobacco type which, after curing, is associated with a spicy and lively sensation. According to 50 the invention, bright tobaccos are tobaccos with a content of reducing sugars of between about 2.5 percent and about 20 percent of dry weight base of the leaf and a total ammonia content of less than about 0.12 percent of dry weight base of the leaf. Reducing sugars comprise for example glucose or fructose. Total ammonia comprises for example ammonia and ammonia salts.

55 Dark tobaccos are tobaccos with a generally large, dark coloured leaves. Throughout the specification, the term "dark tobacco" is used for tobaccos that have been air cured. 60 Additionally, dark tobaccos may be fermented. Tobaccos that are used mainly for chewing, snuff, cigar, and pipe blends are also included in this category. From a sensorial

perspective, dark tobacco is a tobacco type which, after curing, is associated with a smoky, dark cigar type sensation. Dark tobacco is characterized by a low sugar to nitrogen ratio. Examples for dark tobacco are Burley Malawi or other African Burley, Dark Cured Brazil Galpao, Sun Cured or Air Cured Indonesian Kasturi. According to the invention, dark tobaccos are tobaccos with a content of reducing sugars of less than about 5 percent on dry weight basis of the leaf and a total ammonia content of up to about 0.5 percent on dry weight basis of the leaf.

Aromatic tobaccos are tobaccos that often have small, light coloured leaves. Throughout the specification, the term "aromatic tobacco" is used for other tobaccos that have a high aromatic content, for example a high content of essential oils. From a sensorial perspective, aromatic tobacco is a tobacco type which, after curing, is associated with spicy and aromatic sensation. Examples for aromatic tobaccos are Greek Oriental, Oriental Turkey, semi-oriental tobacco but also Fire Cured, US Burley, such as Perique, Rustica, US Burley or Merland.

Additionally, a blend may comprise so called filler tobaccos. Filler tobacco is not a specific tobacco type, but it includes tobacco types which are mostly used to complement the other tobacco types used in the blend and do not bring a specific characteristic aroma direction to the final product. Examples for filler tobaccos are stems, midrib or stalks of other tobacco types. A specific example may be flue cured stems of Flue Cured Brazil lower stalk.

Within each type of tobaccos, the tobacco leaves are further graded for example with respect to origin, position in the plant, colour, surface texture, size and shape. These and other characteristics of the tobacco leaves are used to form a tobacco blend. A blend of tobacco is a mixture of tobaccos belonging to the same or different types such that the tobacco blend has an agglomerated specific characteristic. This characteristic can be for example a unique taste or a specific aerosol composition when heated or burned. A blend comprises specific tobacco types and grades in a given proportion one with respect to the other.

According to the invention, different grades within the same tobacco type may be cross-blended to reduce the variability of each blend component. According to the invention, the different tobacco grades are selected in order to realize a desired blend having specific predetermined characteristics. For example, the blend may have a target value of the reducing sugars, total ammonia and total alkaloids per dry weight base of the homogenized tobacco material. Total alkaloids are for example nicotine and the minor alkaloids including nornicotine, anatabine, anabasine and myosmine.

For example, bright tobacco may comprise tobacco of grade A, tobacco of grade B and tobacco of grade C. Bright tobacco of grade A has slightly different chemical characteristics to bright tobacco of grade B and grade C. Aromatic tobacco may include tobacco of grade D and tobacco of grade E, where aromatic tobacco of grade D has slightly different chemical characteristics to aromatic tobacco of grade E. A possible target value for the tobacco blend, for the sake of exemplification, can be for example a content of reducing sugars of about 10 percent in dry weight basis of the total tobacco blend. In order to achieve the selected target value, a 70 percent bright tobacco and a 30 percent aromatic tobacco may be selected in order to form the tobacco blend. The 70 percent of the bright tobacco is selected among tobacco of grade A, tobacco of grade B and tobacco of grade C, while the 30 percent of aromatic tobacco is selected among tobacco of grade D and tobacco of grade

E. The amounts of tobaccos of grade A, B, C, D, E which are included in the blend depend on the chemical composition of each of the tobaccos of grades A, B, C, D, E so as to meet the target value for the tobacco blend.

According to a second aspect, the invention relates to a homogenized tobacco material comprising a pulp including cellulose fibres and water, a blend of powder of different tobacco types, and a binder, combined together to form a slurry. According to the invention, the tobacco powder has 10 a mean powder size between about 0.03 millimetres and about 0.12 millimetres, the amount of binder is comprised between about 1 percent and about 5 percent in dry weight basis of the slurry and the cellulose fibres added to the tobacco powder are in an amount between about 1 percent 15 and about 3 percent in dry weight basis of the slurry and their mean size is comprised between about 0.2 millimetres and about 4 millimetres.

The cellulose fibres in an amount between about 1 percent and about 3 percent in dry weight basis of the slurry are 20 added to the tobacco powder. Tobacco in itself includes some cellulose fibres, therefore the total amount of cellulose fibres in the homogenized tobacco material may be higher than between about 1 percent and about 3 percent in dry weight basis of the slurry, due to the natural presence of cellulose fibres in the tobacco. However, as discussed in relation to the first aspect, the tobacco fibres are cut in very small pieces due to the tobacco grinding into powder. Preferably, the percentage of cellulose fibres added to the tobacco powder having a mean size comprised between 25 about 1 millimetres and 3 millimetres is equal to 4 times the standard deviation of the size of the cellulose fibres in said pulp. Fibres are natural products having a very wide range of lengths before processing. Preferably, a narrower range than the natural one is obtained by a refining step. Due to the 30 refining step of the method of the invention, the resulting fibres' lengths tend to be very close to the mean. This means that the variations in the lengths of the cellulose fibres are relatively small. The risk of inhomogeneity or defects in the homogenized tobacco material caused by fibres that are 35 much longer than the mean value may be minimized. In particular, long fibres may create so called drappers in the cast tobacco web that frequently create extended inhomogeneous areas in the tobacco web. Preferably, the cellulose fibres added to the tobacco powder are wood cellulose fibres. 40 Alternatively, the source of the cellulose fibres is another plant material such as for example, tobacco, flax or hemp.

Advantageously, the added cellulose fibres are at least 45 partially fibrillated. In a preferred embodiment, the binder comprises guar. The homogenized tobacco material may be 50 cast leaf tobacco. The slurry includes tobacco powder and preferably one or more of fibre particles, aerosol formers, flavours, and binders. Related advantages have already been explained in connection with the inventive method above and, for the sake of simplicity, will not be repeated.

A web of homogenized tobacco material is preferably 55 formed by a casting process of the type generally comprising casting a tobacco slurry onto a moving metal belt. Preferably, the cast web is dried to form a web of homogenized tobacco material and it is then removed from the support surface.

Preferably, the moisture of said cast tobacco material web at casting is between about 60 percent and about 80 percent in weight of the total weight of the cast tobacco web. 60 Preferably, the method for production of a homogenized tobacco material comprises the step of drying said cast tobacco web and winding said cast tobacco web, wherein the moisture of said cast tobacco web at winding is between

about 7 percent and about 15 percent in weight of the total weight of the cast tobacco web.

According to a third aspect, the invention relates to an aerosol-generating article, comprising a portion of the homogenised tobacco material described above.

An aerosol-generating article is an article comprising an aerosol-forming substrate that is capable of releasing volatile compounds that can form an aerosol. An aerosol-generating article may be a non-combustible aerosol-generating article or may be a combustible aerosol-generating article. Non-combustible aerosol-generating article releases volatile compounds without the combustion of the aerosol-forming substrate, for example by heating the aerosol-forming substrate, or by a chemical reaction, or by mechanical stimulus of an aerosol-forming substrate. Combustible aerosol-generating article releases an aerosol by direct combustion of an aerosol-forming substrate, for example as in a conventional cigarette.

The aerosol-forming substrate is capable of releasing volatile compounds that can form an aerosol volatile compound and may be released by heating or combusting the aerosol-forming substrate. In order for the homogenized tobacco material to be used in an aerosol-forming generating article, aerosol formers are preferably included in the slurry that forms the cast leaf. The aerosol formers may be chosen based on one or more of predetermined characteristics. Functionally, the aerosol former provides a mechanism that allows the aerosol former to be volatilize and convey nicotine and/or flavouring in an aerosol when heated above the specific volatilization temperature of the aerosol former.

The invention will be further described, by way of example only, with reference to the accompanying drawings in which:

FIG. 1 shows a flow diagram of a method to produce an homogenized tobacco material according to the invention;

FIG. 2 shows an enlarged view of one of the step of the method of FIG. 1;

FIG. 3 shows a schematic view of an apparatus for performing a step of the method of FIG. 1;

FIG. 4 shows a schematic view of an apparatus for performing another step of the method of FIG. 1;

FIG. 5 shows a schematic view of an apparatus for performing a further step of the method of FIG. 1;

FIG. 6 shows a schematic view of an apparatus for performing a further step of the method of FIG. 1; and

FIG. 7 shows a schematic view of an apparatus for performing a further step of the method of FIG. 1.

With initial reference to FIG. 1, a method for the production of slurry according to the present invention is represented. The first step of the method of the invention is the selection 100 of the tobacco types and tobacco grades to be used in the tobacco blend for producing the homogenized tobacco material. Tobacco types and tobacco grades used in the present method are for example bright tobacco, dark tobacco, aromatic tobacco and filler tobacco.

Only the selected tobacco types and tobacco grades intended to be production of the used for the homogenized tobacco material undergo the processing according to following steps of the method of the invention.

The method includes a further step 101 in which the selected tobacco is laid down. This step may comprise checking the tobacco integrity, such as grade and quantity, which can be for example verified by a bar code reader for product tracking and traceability. After harvesting and curing, the leaf of tobacco is given a grade, which describes for example the stalk position, quality, and colour.

Further, the lay down step 101 might also include, in case the tobacco is shipped to the manufacturing premises for the production of the homogenized tobacco material, de-boxing or case opening of the tobacco boxes. The de-boxed tobacco is then preferably fed to a weighing station in order to weight the same.

Moreover, the tobacco lay down step 101 may include bale slicing, if needed, as the tobacco leaves are normally compressed into bales in shipping boxes for shipping.

10 The following steps are performed for each tobacco type, as detailed below. These steps may be performed subsequently per grade such that only one production line is required. Alternatively, the different tobacco types may be processed in separate lines. This may be advantageous where the processing steps for some of the tobacco types are different. For example, in conventional primary tobacco processes bright tobaccos and dark tobaccos are processed at least partially in separate processes, as the dark tobacco often receives an additional casing. However, according to 15 the present invention, preferably, no casing is added to the blended tobacco powder before formation of the homogenized tobacco web.

Further, the method of the invention includes a step 102 of coarse grinding of the tobacco leaves.

20 According to a variant of the method of the invention, after the tobacco lay down step 101 and before the tobacco coarse grinding step 102, a further shredding step 103 is performed, as depicted in FIG. 1. In the shredding step 103 the tobacco is shredded into strips having a mean size 25 comprised between about 2 millimetres and about 100 millimetres.

30 Preferably, after the shredding step 103, a step of removal of non-tobacco material from the strips is performed (not depicted in FIG. 1).

35 Subsequently, the shredded tobacco is transported towards the coarse grinding step 102. The flow rate of tobacco into a mill to coarse grind the strips of tobacco leaf is preferably controlled and measured.

40 In the coarse grinding step 102, the tobacco strips are reduced to a mean particle size of between about 0.25 millimetres and about 2 millimetres. At this stage, the tobacco particles are still with their cells substantially intact and the resulting particles do not pose relevant transport issues.

45 Preferably, after the coarse grinding step 102, the tobacco particles are transported, for example by pneumatic transfer, to a blending step 104. Alternatively, the step of blending 104 could be performed before the step of coarse grinding 102, or where present, before the step of shredding 103, or, alternatively, between the step of shredding 103 and the step 50 of coarse grinding 102.

55 In the blending step 104, all the coarse grinded tobacco particles of the different tobacco types selected for the tobacco blend are blended. The blending step 104 therefore is a single step for all the selected tobacco types. This means that after the step of blending there is only need for a single process line for all of the different tobacco types.

60 In the blending step 104, preferably mixing of the various tobacco types in particles is performed. Preferably a step of measuring and controlling one or more of the properties of the tobacco blend is performed. According to the invention, the flow of tobacco may be controlled such that the desired blend according to a pre-set target value or pre-set target values is obtained. For example, it may be desirable that the 65 blend includes bright tobacco 1 at least for about 30 percent in dry weight of the total tobacco in the blend, and that dark tobacco 2 and aromatic tobacco 3 are comprised each in a

## 11

percentage between about 0 percent and about 40 percent in dry weight basis of the total tobacco in the blend, for example about 35 percent. More preferably, also filler tobacco 4 is introduced in a percentage between about 0 percent and about 20 percent in dry weight basis of the total tobacco in the blend. The flow rate of the different tobacco types is therefore controlled so that this ratio of the various tobacco types is obtained. Alternatively, where the coarse grinding step 102 is done subsequently for the different tobacco leafs used, the weighing step at the beginning of the step 102 determines the amount of tobacco used per tobacco type and grade instead of controlling its flow rate.

In FIG. 2, the introduction of the various tobacco types during the blending step 104 is shown.

It is to be understood that each tobacco type could be itself a sub-blend, in other words, the "bright tobacco type" could be for example a blend of Virginia tobacco and Brazil flue-cured tobacco of different grades.

After the blending step 104, a fine grinding step 105, to a tobacco powder mean size of between about 0.03 millimetres and about 0.12 millimetres is performed. This fine grinding step 105 reduces the size of the tobacco down to a powder size suitable for the slurry preparation. After this fine grinding step 105, the cells of the tobacco are at least partially destroyed and the tobacco powder may become sticky.

The so obtained tobacco powder can be immediately used to form the tobacco slurry. Alternatively, a further step of storage of the tobacco powder, for example in suitable containers may be inserted (not shown).

The steps of tobacco blending and grinding tobacco for the formation of a homogenized tobacco material according to FIG. 1 are performed using an apparatus for the grinding and blending of tobacco 200 depicted schematically in FIG. 3. The apparatus 200 includes a tobacco receiving station 201, where accumulating, de-stacking, weighing and inspecting the different tobacco types takes place. Optionally, in case the tobacco has been shipped into cartons, in the receiving station 201 removal of cartons containing the tobacco is performed. The tobacco receiving station 201 also optionally comprises a tobacco bale splitting unit.

In FIG. 3 only a production line for one type of tobacco is shown, but the same equipment may be present for each tobacco type used in the homogenised tobacco material web according to the invention, depending on when the step of blending is performed. Further the tobacco is introduced in a shredder 202 for the shredding step 103. Shredder 202 can be for example a pin shredder. The shredder 202 is preferably adapted to handle all sizes of bales, to loosen tobacco strips and shred strips into smaller pieces. The shreds of tobacco in each production line are transported, for example by means of pneumatic transport 203, to a mill 204 for the coarse grinding step 102. Preferably a control is made during the transport so as to reject foreign material in the tobacco shreds. For example, along the pneumatic transport of shredded tobacco, a string removal conveyor system, heavy particle separator and metal detector may be present, all indicated with 205 in the appended drawing.

Mill 204 is adapted to coarse grind the tobacco strips up to a size of between about 0.25 millimetres and about 2 millimetres. The rotor speed of the mill can be controlled and changed on the basis of the tobacco shreds flow rate.

Preferably, a buffer silo 206 for uniform mass flow control, is located after the coarse grinder mill 204. Furthermore, preferably mill 204 is equipped with spark detectors and safety shut down system 207 for safety reasons.

## 12

From the mill 204, the tobacco particles are transported, for example by means of a pneumatic transport 208, to a blender 210. Blender 210 preferably includes a silo in which an appropriate valve control system is present. In the 5 blender, all tobacco particles of all the different types of tobacco which have been selected for the predetermined blend are introduced. In the blender 210, the tobacco particles are mixed to a uniform blend. From the blender 210, the blend of tobacco particles is transported to a fine 10 grinding station 211.

Fine grinding station 211 is for example an impact classifying mill with suitable designed ancillary equipment to produce fine tobacco powder to the right specifications, that is, to a tobacco powder between about 0.03 millimetres and about 0.12 millimetres. After the fine grinding station 211, a 15 pneumatic transfer line 212 is adapted to transporting the fine tobacco powder to a buffer powder silo 213 for continuous feed to a downstream slurry batch mixing tank where the slurry preparation process takes place.

The method for the production of a homogenized tobacco material of FIG. 1 further includes a step of suspension preparation 106. The suspension preparation step 106 preferably comprises mixing an aerosol-former 5 and a binder 6 25 in order to form a suspension. Preferably, the aerosol-former 5 comprises glycerol and the binder 6 comprises guar. The step of forming a suspension 106 of binder in aerosol-former includes the steps of loading the aerosol-former 5 and the binder 6 in a container and mixing the two. Preferably, the resulting suspension is then stored before being introduced in the slurry. Preferably, the glycerol is added to the guar in two steps, a first amount of glycerol is mixed with guar and a second amount of glycerol is then injected in the transport pipes, so that glycerol is used to clean the 30 processing line, avoiding hard-to-clean points within the line. A slurry preparation line 300 adapted to perform the suspension of binder in aerosol-former as per step 106 of the invention is depicted in FIG. 4.

The slurry preparation line 300 includes an aerosol-former, 40 such as glycerol, bulk tank 301 and a pipe transfer system 302 having a mass flow control system 303 adapted to transfer the aerosol-former 5 from the tank 301 and to control its flow rate. Further, the slurry preparation line 300 45 comprises a binder handling station 304 and a pneumatic transport and dosing system 305 to transport and weight the binder 6 received at the station 304.

Aerosol-former 5 and binder 6 from tank 301 and handling station 304, respectively, are transported to a mixing tank, or more than a mixing tank, 306, part of the slurry preparation line 300, designed to mix binder 6 and aerosol-former 5 uniformly.

The method to realize the homogenized tobacco material includes a step of preparing a cellulose pulp 107. The pulp preparation step 107 preferably comprises mixing cellulose 55 fibres 7 and water 8 in a concentrated form, optionally storing the pulp so obtained and then diluting the concentrated pulp before forming the slurry. The cellulose fibres, for example in boards or bags, are loaded in a pulper and then liquefied with water. The resulting water-cellulose 60 solution may be stored at different densities, however preferably the pulp which is the result of the step 107 is "concentrate". Preferably, "concentrate" means that the total amount in the cellulose fibres in the pulp is between about 3 percent and 5 percent of the total pulp weight before dilution. Preferred cellulose fibres are soft wood fibres. Preferably, the total amount of cellulose fibres in the slurry 65 in dry weight is between about 1 percent and about 3

## 13

percent, preferably, between about 1.2 percent and about 2.4 percent in dry weight of the slurry.

Preferably, the step of mixing of water and cellulose fibres lasts between about 20 and about 60 minutes, advantageously at a temperature comprised between about 15 degrees Celsius and about 40 degrees Celsius.

The storage time, if storage of the pulp is performed, may preferably vary between about 0.1 day and about 7 days.

Advantageously, water dilution takes place after the step of storing of the concentrated pulp. Water is added to the concentrated pulp in such an amount that the cellulose fibres are less than about 1 percent of the total weight of the pulp. For example a dilution of a factor comprised between about 3 and about 20 can take place. Further, an additional step of mixing may take place, which comprises mixing the concentrated pulp and the added water. The additional mixing step preferably lasts between about 120 minutes and about 180 minutes at a temperature between about 15 degrees Celsius and about 40 degrees Celsius, more preferably at a temperature of between about 18 degrees Celsius and about 25 degrees Celsius.

All tanks and transfer pipes for cellulose fiber, guar and glycerol are preferably designed to be as optimally short as possible to reduce transfer time, minimize waste, avoid cross contamination and facilitate ease of cleaning. Further, preferably, the transfer pipes for cellulose fiber, guar and glycerol are as straight as possible, to allow a swift and uninterrupted flow. In particular for the suspension of binder in the aerosol-former, turns in the transfer pipe could otherwise result in areas of low flow rate or even standstill, which in turn can be areas where gelling can occur and with that potentially blockages within the transfer pipes. As mentioned before, those blockages can lead to the need for cleaning and standstill of the entire manufacturing process.

Preferably, after the step of pulp preparation 107, an optional step of fibres' fibrillation is performed (not depicted in FIG. 1).

An apparatus 400 to perform the method step 107 of the pulp formation is depicted in FIG. 5. FIG. 5 schematically depicts a cellulose fibre feeding and preparation line 400 comprising a feeding system 401, preferably adapted to handle cellulose fibres 7 in bulk form, such as board/sheets or fluffed fibres, and a pulper 402. The feeding system 401 is adapted to direct the cellulose fibres to the pulper 402, which is in turn adapted to disperse the received fibres uniformly.

The pulper 402 includes a temperature control unit 401a so that the temperature in the pulper is kept within a given temperature interval, and a rotational speed control unit 401b, so that the speed of an impeller (not shown) present in the pulper 402 is controlled and kept preferably comprised between about 5 rpm and about 35 rpm.

The cellulose fibre feeding and preparation line 400 further comprises a water line 404 adapted to introduce water 8 in the pulper 402. A flow rate controller 405 to control the flow rate of water introduced in pulper 402 is preferably added in the water line 404.

The cellulose fibre feeding and preparation line 400 may also further comprise a fibre refiner system 403 to treat and fibrillate fibres, so that long fibres and nested fibres are removed, and a uniform fibre distribution is obtained.

Preferably, the mean size of the cellulose fibres at the end of the pulping and refining step is comprised between about 0.2 millimetres and about 4 millimetres, more preferably between about 1 millimetre and about 3 millimetres.

The mean size is considered to be the mean length. Each length of the fibre is calculated following the framework of

## 14

the fibre, therefore it is the real developed length of the fibre. The mean fibre length is calculated per number of fibres, for example it may be calculated on 5.000 fibers.

Measured objects are considered a fibres if their length and width are comprised within:

$$200 \mu\text{m} < \text{length} < 10.000 \mu\text{m}$$

$$5 \mu\text{m} < \text{width} < 75 \mu\text{m}$$

In order to calculate the mean fibre length, the MorFi Compact fibre analyzer on fibers produced by Tech Pap SAS can be used.

The analysis is performed for example putting the fibres in a solution, so as to form an aqueous fibrous suspension. Preferably, deionized water is used and no mechanical mixing is applied during sample preparation. Mixing is performed by the fibre analyzer. Preferably, measurements are performed on fibres which have stayed at least 24 hours at about 22 degrees Celsius and about 50 percent relative humidity.

Downstream the fibre refiner system 403, the cellulose fibre feeding and preparation line 400 may comprise a cellulose buffer tank 407 connected to the fibre refiner system 403 to store the high consistency fibre solution coming out of the system 403.

At the end of cellulose fibre feeding and preparation line 400, a cellulose dilution tank 408 in which pulp is diluted is preferably present and connected to cellulose buffer tank 407. The cellulose dilution tank 408 is adapted to batch out cellulose fibres of right consistency for subsequent slurry mixing. Water for dilution is introduced in tank 408 via a second water line 410.

The method to form a slurry according to the invention further comprises a step of slurry formation 108, where the suspension 9 of binder in aerosol-former obtained in step 106, the pulp 10 obtained in step 107 and the tobacco powder blend 11 obtained in step 104 are combined together.

Preferably, the step of slurry formation 108 comprises first a step of introduction in a tank of the suspension 9 of binder in aerosol-former and of the cellulose pulp 10. Afterwards, the tobacco powder blend 11 is introduced as well. Preferably, the suspension 9, the pulp 10 and the tobacco powder blend 11 are suitably dosed in order to control the amount of each of them introduced in the tank. The slurry is prepared according to specific proportion among its ingredients. Optionally, also water 8 is added as well.

Preferably, the step of slurry formation 108 also comprises a mixing step, where all the slurry ingredients are mixed together for a fixed amount of time. In a further step of the method according to the invention, the slurry is then transferred to a following casting step 109 and drying step 110.

An apparatus 500 for the slurry formation adapted to realize step 108 of the method of the invention is schematically depicted in FIG. 6. Apparatus 500 includes a mixing tank 501 where cellulose pulp 10 and suspension 9 of binder in aerosol-former are introduced. Further, the tobacco powder blend 11 from the blending and grinding line is fine-ground and dosed into the mixing tank 501 in specified quantity to prepare the slurry.

For example, the tobacco powder blend 11 may be contained in a tobacco fine powder buffer storage silo to ensure continuous upstream powder operation and meeting demand of slurry mixing process. Tobacco powder is transferred to the mixing tank 501 preferably by means of a pneumatic transfer system (not shown).

## 15

The apparatus **500** further comprises preferably a powder dosing/weighing system (also not shown) to dose required amount of the slurry's ingredients. For example, the tobacco powder may be weighted by a scale (not shown) or weighting belt (not shown) for precise dosing. The mixing tank **501** is specially designed to mix the dry and liquid ingredients to form a homogenous slurry. The slurry mixing tank preferably comprises a cooler (not shown), such as water jacket wall to allow water cooled on the external walls of the mixing tank **501**. The slurry mixing tank **501** is further equipped with one or more sensors (not shown) such as a level sensor, a temperature probe and a sampling port for control and monitoring purpose. Mixing tank **501** has an impeller **502** adapted to ensure uniform mixing of the slurry, in particular adapted to transfer slurry from the external walls of the tank to the internal part of the tank or vice-versa. The speed of the impeller can be preferably controlled by means of a dedicated controlling unit. Mixing tank **501** also includes a water line for the introduction of water **8** at a controlled flow rate.

Preferably, mixing tank **501** includes two separated tanks, one downstream to the other in the flow of slurry, one tank for preparing the slurry and the second tank with slurry for transfer to provide continuous slurry supply to a casting 25

The method of the invention to produce a homogenized tobacco web includes further a casting step **109** in which the slurry prepared in step **108** is cast in a continuous tobacco web onto a support. The casting step **109** includes transferring the slurry from the mixing tank **501** to a casting box. Further, it preferably includes monitoring the level of slurry in the casting box and the moisture of the slurry. Then, the casting step **109** includes casting, preferably by means of a casting blade, the slurry onto a support, such as a steel conveyor. Further, in order to obtain a final homogenized tobacco web for the use in an aerosol-formed article, the method of the invention includes a drying step **110** in which the cast web of homogenized tobacco material is preferably dried. The drying step **110** includes drying the cast web, by means of steam and heated air. Preferably the drying with steam is performed on the side of the cast web in contact with the support, while the drying with heated air is performed on the free side of the cast web.

An apparatus for performing the steps of casting **109** and drying **110** is schematically depicted in FIG. 7. The casting and drying apparatus **600** includes a slurry transfer system **601**, such as a pump, preferably having a flow control, and a casting box **602** to which the slurry is transferred by the pump. Preferably, casting box **602** is equipped with level control **603** and a casting blade **604** for the casting of the slurry into a continuous web of homogenized tobacco material. Casting box **602** may also comprise a density control device **605** to control the density of the cast web.

A support, such as a stainless steel belt conveyor **606**, receives the slurry cast by the casting blade **604**.

Casting and drying apparatus **600** also includes a drying station **608** to dry the cast web of slurry. Drying station **608** comprises a steam heating **609** and top air drying **610**.

Preferably, at the end of the casting step **109** and of the drying step **110**, the homogenized tobacco web is removed from the support **606**. Doctoring of the cast web after the drying station **608** at the right moisture content is preferably performed.

The cast web goes preferably through a secondary drying process to remove further moisture content of the web to reach moisture target or specification.

## 16

After the drying step **110**, the cast web is preferably wound in one or more bobbins in a winding step **111**, for example to form a single master bobbin. This master bobbin may be then used to perform the production of smaller bobbins by slitting and small bobbin forming process. The smaller bobbin may then be used for the production of an aerosol-generating article (not shown).

The invention claimed is:

1. Method for the preparation of a homogenized tobacco material, said method comprising:

pulping and refining cellulose fibres to obtain fibres having a mean size comprised between about 0.2 millimetres and about 4 millimetres;

grinding a blend of tobacco of one or more tobacco types to a tobacco powder having a mean size lower than about 0.12 millimetres;

combining the pulp with the tobacco powder blend of different tobacco types and with a binder in an amount comprised between about 1 percent and about 5 percent in dry weight basis of the total weight of the homogenized tobacco material, and an aerosol former in an amount comprised between about 5 percent and about 30 percent in dry weight basis of the total weight of the homogenized tobacco material so as to form a slurry; homogenizing the slurry; and

forming the homogenized tobacco material from the slurry.

2. Method according to claim 1, wherein the step of pulping and refining comprises a step of fibrillating the cellulose fibres at least in part.

3. Method according to claim 2, comprising: vibrating the slurry.

4. Method according to claim 1, comprising: vibrating the slurry.

5. Method according to claim 1, wherein the step of pulping and refining comprises a step of pulping and refining cellulose fibres to obtain fibres having a mean size comprised between about 1 millimetre and about 3 millimetres.

6. Method according to claim 5, wherein the step of pulping and refining comprises the steps of:

forming a concentrated pulp wherein the amount of the cellulose fibres is between about 3 percent and about 5 percent of the total weight of the concentrated pulp; diluting said concentrated pulp wherein the amount of cellulose fibres is below about 1 percent of the total weight of the diluted pulp.

7. Method according to claim 1, wherein the step of pulping and refining comprises the steps of:

forming a concentrated pulp wherein the amount of the cellulose fibres is between about 3 percent and about 5 percent of the total weight of the concentrated pulp; diluting said concentrated pulp wherein the amount of cellulose fibres is below about 1 percent of the total weight of the diluted pulp.

8. Method according to claim 1, wherein the step of forming a homogenized tobacco material from the slurry comprises the steps of:

casting a web of the slurry; and drying said cast web.

9. Method according to claim 1, wherein said step of grinding tobacco of one or more tobacco types comprises blending one or more of the following tobaccos:

Bright tobacco;  
Dark tobacco;  
Aromatic tobacco;  
Filler tobacco.

**17**

10. Aerosol-generating article, comprising a portion of the homogenised tobacco material realized according to the method of claim 1.

11. A homogenized tobacco sheet comprising a pulp comprising refined cellulose fibres and water; a blend of powder of different tobacco types having a mean powder size lower than about 0.12 millimetres; a binder in a quantity between about 1 percent and about 5 percent in dry weight of the homogenized tobacco sheet; an aerosol former in a quantity between about 5 percent and about 30 percent in dry weight basis of the homogenized tobacco sheet; wherein said cellulose fibres added to the tobacco powder blend are in an amount comprised between about 1 percent and about 3 percent dry weight basis of the total weight of the homogenized tobacco sheet and their mean size is comprised between about 0.2 millimetres and about 4 millimetres.

**18**

12. Homogenized tobacco sheet according to claim 11, wherein the mean size of the cellulose fibres added to the tobacco powder blend is comprised between about 1 millimetre and about 3 millimetres.

13. Homogenized tobacco sheet according to claim 11, wherein a percentage of cellulose fibres added to the tobacco powder blend having a mean size comprised between about 1 millimetres and 3 millimetres is equal to 4 times a standard deviation of the size of the cellulose fibres in said pulp.

14. Homogenized tobacco sheet according to claim 11, wherein the cellulose fibres added to the tobacco powder blend comprise wood cellulose fibres.

15. Homogenized tobacco sheet according to claim 11, wherein the cellulose fibres added to the tobacco powder blend are at least partially fibrillated.

16. Homogenized tobacco material according to claim 11, wherein the binder includes guar.

17. Aerosol-generating article, comprising a portion of the homogenised tobacco material of claim 11.

\* \* \* \* \*